

# UNITED STATES PATENT OFFICE.

LEON McCULLOCH, OF WILKINSBURG, PENNSYLVANIA, ASSIGNOR TO WESTINGHOUSE ELECTRIC AND MANUFACTURING COMPANY, A CORPORATION OF PENNSYLVANIA.

## ELECTRIC RESISTANCE ELEMENT.

1,365,331.

Specification of Letters Patent. Patented Jan. 11, 1921.

No Drawing.

Application filed June 8, 1916. Serial No. 102,481.

To all whom it may concern:

Be it known that I, LEON McCULLOCH, a citizen of the United States, and a resident of Wilkinsburg, in the county of Allegheny and State of Pennsylvania, have invented a new and useful Improvement in Electric Resistance Elements, of which the following is a specification.

My invention relates to resistance elements for use in electric apparatus, such as rheostats, heating devices and the like, and it has for its general object to provide resistance elements of great durability under service conditions.

More particularly, my invention aims to utilize resistance conductors which have not heretofore been practically available for this use on account of their rapid deterioration when subjected to electric current under operating conditions.

Many conductors of electricity are suitable for use as resistance elements, so far as their electrical characteristics are concerned, but relatively few of such conductors have heretofore been of practical utility because of the degree to which most of them become oxidized at elevated temperatures. Numerous attempts have been made to coat resistors with enamels, glazes or cements, but this expedient has been satisfactory only in the case of resistors intended for operation at relatively low temperatures, on account of the fact that the protective coatings must be applied in liquid form or must be liquefied during the coating process, and, when the coated resistor is heated, it has been found that the coating will again liquefy and drop from the conductor.

According to my present invention, I produce satisfactory coated resistors by utilizing a class of coating materials which I have found to possess the property of softening under moderate heat, but melting to complete fluidity only at temperatures above the temperatures present in the ordinary forms of electric resistance apparatus. This peculiar property of the coatings which I employ makes it possible, not only to apply permanent coatings to conductors which are afterward to be highly heated, but to provide a coating which is flexible and not likely to crack under variations of temperature, as most coating materials will do.

The coating substances which I prefer to employ are compounds of boron, particularly its oxygen compounds such as the borates, metaborates and oxids. Many conducting materials are suitable for use in connection with these protective coatings, such, for example, as nickel steel and other iron alloys, as well as non-ferrous alloys and all other conducting substances having high specific resistance and mechanical strength. Specific examples of suitable resistance alloys are nickel-steel containing about 30% of nickel, cupro-nickel composed of about 60% copper and 40% nickel, and the common varieties of German silver. I shall illustrate my invention by describing the treatment of resistors to produce coatings of boron trioxid upon them, it being understood, however, that my invention is by no means restricted to the use of this particular conductor or this particular coating.

According to one method of carrying out this process, I prepare an aqueous solution of ammonium orthoborate, preferably a saturated, or at least a concentrated, solution and preferably with the addition of an excess of ammonium hydroxid. This solution may be at once applied to a portion or all of the surface of the resistor to be coated, either by dipping or by brushing, or it may be mixed with a small amount of any suitable filler such as kaolin, metallic oxids, or clays of the bentonite type. The coating mixture may be applied to the resistance material before the material is given its final form, but I find it convenient to first shape the resistor or mount it upon an insulating support and to apply the coating as a final step. For example, resistance elements for heating apparatus such as sad irons and percolators are commonly formed by winding a wire or ribbon of a resistance conductor upon an insulating support of mica, lava or the like, and, in such cases, the coating material may be applied to the entire structure.

After the preliminary coating described above is applied to the resistor, the latter is subjected to heat to decompose the ammonium borate and to drive off the ammonia and water from the coating. This heat treatment may be suitably carried out at a temperature of about 500° C. and be con-

tinued until substantially all the ammonia and water are expelled, leaving a coating of boron trioxid which is inert to the metal. The resistor may then be used without further treatment, or an additional coating of refractory cement may be applied over the boric oxid coating as a mechanical protection and also to prevent free access of moisture to the boric oxid.

- 10 A suitable solution for use in carrying out the above process may be made by dissolving about 65 grams of an ammonium borate in 100 grams of hot water and adding about 20 cubic centimeters of concentrated ammonium hydroxid. A smaller proportion of ammonium borate may be employed, but I find that better results are obtained if the solution is concentrated or even saturated.

The boric oxid coating may be obtained in 20 a number of ways in addition to the method described above. For example, the boric oxid, in powdered form, may be sprinkled upon the resistor to be coated, which is then heated to soften the boric oxid sufficiently 25 to permit it to be spread in an even layer over the surface of the resistor. As stated above, the boric oxid will soften and flow sufficiently for spreading but it will not fully melt until a temperature much above 30 500° C. is reached. The boric oxid coating may also be obtained by the application of boric acid, either in dry powdered form or in solution or suspension in water, alcohol, glycerin, turpentine or any other suitable 35 vaporizable menstruum. For example, boric acid, ammonium borate, or some other substance yielding boric oxid upon heating, may be ground to a fine paste in a vehicle such as water, which should be insufficient in 40 quantity to dissolve the powdered material. One suitable paste of this class is made by triturating about 700 grams of ammonium orthoborate in a mixture of about 950 cubic centimeters of water and about 150 cubic 45 centimeters of ammonium hydroxid, sp. gr. 0.92. These proportions may be varied within wide limits. The flowing properties of these pastes may be increased by the addition of a small amount, two or three per 50 cent., of a clay of the bentonite type.

In addition to boron trioxid, other boron compounds are suitable for use according to my present invention, for example, the metallic borates, such as lead borate, sodium borate, sodium metaborate and borax.

Some of the boron compounds which I have mentioned possess the advantage, in addition to their behavior under the action of heat, that they have but little fluxing 60 effect upon other insulating materials such as mica, and may therefore be used in contact with them. Furthermore, these coatings, while belonging to the class of materials in which electric resistivity decreases 65 with increase in temperature, exhibit this

property but little within the range of temperatures encountered in ordinary resistance apparatus.

One advantage of the use of some low-melting compound to surround the heating element embedded between mica plates is the fact that the heat conductivity of the insulation is considerably increased, causing the resistor to operate at a lower temperature for the same heat output. All of these properties combine to increase the efficiency of resistors provided with these coatings. In view of the considerable range of materials and process steps which may be employed without exceeding the limits of my invention, it is to be understood that the scope of my invention is limited only by that of the appended claims.

I claim as my invention:

1. An electric resistance element comprising a conductor of electricity having at least a portion of its surface covered with a coating material that softens, but does not fully melt, at the operating temperature of the said resistance element.

2. An electric resistance element comprising a conductor of electricity having at least a portion of its surface covered with a coating material that softens at a temperature below 500° C. but melts at a temperature above 500° C.

3. An electric resistance element comprising a conductor of electricity having at least a portion of its surface covered with a coating consisting essentially of a compound of boron.

4. An electric resistance element comprising a conductor of electricity having at least a portion of its surface covered with a coating consisting essentially of an oxygen compound of boron.

5. An electric resistance element comprising a conductor of electricity having at least a portion of its surface covered with a coating comprising a compound of boron that softens, but does not fully melt, at a temperature below the operating temperature of the said resistance element.

6. An electric resistance element comprising a conductor of electricity having at least a portion of its surface covered with a coating consisting essentially of boron trioxid.

7. An electric resistance element comprising a conductor of electricity having at least a portion of its surface covered with a coating comprising a compound of boron, the said coating being covered with cementitious material.

8. An electric resistance element comprising a conductor of electricity having at least a portion of its surface covered with a coating comprising a compound of boron that softens, but does not fully melt at a temperature below the operating temperature of the

said resistance element, the said coating being covered with cementitious material.

9. An electric resistance element comprising a conductor of electricity having at least 5 a portion of its surface covered with a coating comprising an oxygen compound of boron, the said coating being covered with cementitious material.

10. An electric resistance element comprising a conductor of electricity having at 10 least a portion of its surface covered with a coating comprising boron trioxid, the said coating being covered with cementitious material.

15 11. An electric resistance element comprising a body of nickel steel having at least a portion of its surface covered with a coating comprising a compound of boron.

12. An electric resistance element comprising 20 a body of nickel steel having at least a portion of its surface covered with a coating comprising a compound of boron that softens, but does not melt, at a temperature below 500° C.

25 13. An electric resistance element comprising a body of nickel steel having at least a portion of its surface covered with a coating comprising an oxygen compound of boron.

40 14. An electric resistance element comprising a body of nickel steel having at least

a portion of its surface covered with a coating comprising boron trioxid.

15. An electric resistance element comprising a conductor of electricity having at 35 least a portion of its surface covered with a coating comprising an oxygen compound of boron and a small proportion of bentonite.

16. An electric-resistance element comprising a body of nickel steel with an 40 oxidization-preventing coating of a compound of boron.

17. An electric-resistance element comprising a conductor of electricity, having at 45 least a portion of its surface covered with a coating comprising a compound of boron and a small amount of a filler.

18. An electric-resistance element comprising a conductor of electricity, having at 50 least a portion of its surface covered with a coating of a compound of boron together with a small amount of a clay as a filler.

19. An electric-resistance element comprising a conductor of electricity, having at 55 least a portion of its surface covered with a coating comprising a compound of boron together with substantially 2 to 8% of bentonite.

In testimony whereof I have hereunto subscribed my name this 26th day of May, 1916. 60

LEON McCULLOCH.